

# UNITED STATES PATENT OFFICE.

JOHN A. BAUMGARDNER, OF DETROIT, MICHIGAN.

## MATERIAL FOR THE CEMENTATION OR CASEHARDENING OF IRON AND STEEL.

No Drawing.

Application filed October 7, 1921. Serial No. 503,153.

To all whom it may concern:

Be it known that I, JOHN A. BAUMGARDNER, a citizen of the United States, and resident of Detroit, county of Wayne, State of Michigan, have made a new and useful Invention in a Material for the Cementation or Casehardening of Iron and Steel, which is fully set forth in the following description.

10 The most commonly used mixtures for this purpose consist of a carbonaceous material, such as charcoal, coke, charred leather, lampblack, etc., as a base, combined with one or more of the carbonates of the 15 alkali or the alkaline earth metals as energizer. The theory of the carburizing action of such mixtures is that it is due to the action of carbon monoxide gas generated when they are heated to the carburizing 20 temperature.

At the same time, it is generally conceded that hydrocarbon gases are energetic carburizing agents.

My invention consists in the use of an 25 acetate of the alkali or the alkaline earth metals as an energizer, which energizer will, according to my theory, in itself perform the functions of the carbonates in the above mixtures and at the same time supplement 30 this action by the formation of hydrocarbon gases.

For example, I take wood charcoal and coke, either singly or combined, to which I add 5 to 10 percent by weight calcium 35 acetate, although I do not restrict myself to these percentages. My theory is that on heating, this energizer decomposes into cal-

cium carbonate and acetone which latter subsequently breaks down into hydrocarbon gases and other compounds. Thus it 40 has a double action and I have found it to be more effective than calcium carbonate as an energizer.

I admit that it has been suggested to use barium acetate as an energizer in connection with charcoal in case hardening. 45 However, barium acetate decomposes at a relatively low temperature, very much lower than calcium acetate. The result is that acetone, on which I rely to break 50 down and form the hydrocarbon gases, escapes before the case hardening temperature is reached. With calcium acetate, which decomposes at a very much higher temperature and with the other alkali and 55 alkaline earth metals, such as potassium acetate and sodium acetate, the decomposing point is even higher than with calcium acetate, and I find that the acetone, which breaks down into the hydrocarbon gases, 60 remains for part or all the carburization step.

Having thus fully set forth the nature of my invention, what I claim as new is,—

1. A cementation or casehardening mixture containing a carbonaceous material and calcium acetate.

2. A cementation, or case hardening mixture containing a carbonaceous material, and an acetate of the alkali or alkaline earth metals having a decomposing temperature at least as high as calcium acetate.

In testimony whereof I affix my signature.

JOHN A. BAUMGARDNER.